# EUROPEAN PATENT SPECIFICATION

(11) **EP 2 503 573 B1**
(45) Date of publication and mention of the grant of the patent: **11.06.2014**
(21) Application number: 11765495.4
(22) Date of filing: 28.03.2011
(51) Int. Cl.: H01F 41/02, B22F 1/00, B22F 1/02, C22C 33/02, C22C 38/00, H01F 1/053, H01F 1/08, H01F 1/057

(54) **MANUFACTURING METHOD FOR PERMANENT MAGNET**
VERFAHREN ZUR HERSTELLUNG EINES PERMANENTMAGNETEN
PROCÉDÉ DE FABRICATION D'UN AIMANT PERMANENT

(30) Priority: 31.03.2010 JP 2010084457
(43) Date of publication of application: 26.09.2012
(73) Proprietor: Nitto Denko Corporation, Ibaraki-shi, Osaka 567-8680 (JP)
(72) Inventor: OZEKI Izumi, Ibaraki-shi Osaka 567-8680 (JP); KUME Katsuya, Ibaraki-shi Osaka 567-8680 (JP); HIRANO Keisuke, Ibaraki-shi Osaka 567-8680 (JP); OMURE Tomohiro, Ibaraki-shi Osaka 567-8680 (JP); TAIHAKU Keisuke, Ibaraki-shi Osaka 567-8680 (JP); OZAKI Takashi, Ibaraki-shi Osaka 567-8680 (JP)
(74) Representative: Grünecker, Kinkeldey, Stockmair & Schwanhäusser
(86) International application number: PCT/JP2011/057576
(87) International publication number: WO 2011/125595

(56) References cited:
- WO-A1-2009/128459
- JP-A- 2001 020 065
- JP-A- 2005 039 089
- JP-A- 2005 097 697
- JP-A- 2005 197 299
- JP-A- 2009 259 956
- US-A1- 2004 187 963
- US-A1- 2005 133 117

## Description

### TECHNICAL FIELD

The present invention relates to a manufacturing method for a permanent magnet.

### BACKGROUND ART

In recent years, a decrease in size and weight, an increase in power output and an increase in efficiency have been required in a permanent magnet motor used in a hybrid car, a hard disk drive, or the like. To realize such a decrease in size and weight, an increase in power output and an increase in efficiency in the permanent magnet motor mentioned above, film-thinning and a further improvement in magnetic performance are required of a permanent magnet to be buried in the permanent magnet motor. Meanwhile, as permanent magnet, there have been known ferrite magnets, Sm-Co-based magnets, Nd-Fe-B-based magnets, Sm₂Fe₁₇Nₓ-based magnets or the like. As permanent magnet for permanent magnet motor, there are typically used Nd-Fe-B-based magnets due to remarkably high residual magnetic flux density.

As method for manufacturing a permanent magnet, a powder sintering process is generally used. In this powder sintering process, raw material is coarsely milled first and furthermore, is finely milled into magnet powder by a jet mill (dry-milling) method. Thereafter, the magnet powder is put in a mold and pressed to form in a desired shape with magnetic field applied from outside. Then, the magnet powder formed and solidified in the desired shape is sintered at a predetermined temperature (for instance, at a temperature between 800 and 1150 degrees Celsius for the case of Nd-Fe-B-based magnet) for completion.

On the other hand, as to Nd-based magnets such as Nd-Fe-B magnets, poor heat resistance is pointed to as defect. Therefore, in case a Nd-based magnet is employed in a permanent magnet motor, continuous driving of the motor brings the magnet into gradual decline of coercive force and residual magnetic flux density. Then, in case of employing a Nd-based magnet in a permanent magnet motor, in order to improve heat resistance of the Nd-based magnet, Dy (dysprosium) or Tb (terbium) having high magnetic anisotropy is added to further improve coercive force.

Meanwhile, the coercive force of a magnet can be improved without using Dy or Tb. For example, it has been known that the magnetic performance of a permanent magnet can be basically improved by making the crystal grain size in a sintered body very fine, because the magnetic characteristics of a magnet can be approximated by a theory of single-domain particles. Here, in order to make the grain size in the sintered body very fine, a particle size of the magnet raw material before sintering also needs to be made very fine. However, even if the magnet raw material finely milled into a very fine particle size is compacted and sintered, grain growth occurs in the magnet particles at the time of sintering. Therefore, after sintering, the crystal grain size in the sintered body increases to be larger than the size before sintering, and as a result, it has been impossible to achieve a very fine crystal grain size. In addition, if the crystal grain has a larger size, the domain walls created in a grain easily move, resulting in drastic decrease of the coercive force.

Therefore, as a means for inhibiting the grain growth of magnet particles, there is considered a method of adding a substance for inhibiting the grain growth of the magnet particles (hereinafter referred to as a grain growth inhibitor), to the magnet raw material before sintering. According to this method, for example, the surface of a magnet particle before sintering is coated with the grain growth inhibitor such as a metal compound whose melting point is higher than the sintering temperature, which makes it possible to inhibit the grain growth of magnet particles at sintering. In JP Laid-open Patent Application Publication No. 2004-250781, for example, phosphorus is added as grain growth inhibitor to the magnet powder. Patent document 3 discloses a method, wherein a slurry is prepared by mixing a dry-milled magnet material with a rust preventive oil to inhibit the grain growth of the magnet particles at the time of sintering.

### PRIOR ART DOCUMENT

### PATENT DOCUMENT

Patent document 1: Japanese Registered Patent Publication No. 3298219 (pages 4 and 5)
Patent document 2: Japanese Laid-Open Patent Application Publication No. 2004-250781 (pages 10-12, FIG. 2)
Patent document 3: International Patent Application Publication No. WO 2009/128459 A1

### DISCLOSURE OF THE INVENTION

### PROBLEM TO BE SOLVED BY THE INVENTION

However, as described in Patent Document 2, if the grain growth inhibitor is added to the magnet powder in a manner being previously contained in an ingot of the magnet raw material, the grain growth inhibitor is dispersed in the magnet particles, instead of being settled on the surfaces of the magnet particles. As a result, the grain growth during sintering cannot be sufficiently inhibited, and also the residual magnetic flux density is lowered. Furthermore, even in a case where each magnet particle after sintering can be successfully made very fine by the inhibition of grain growth, exchange interaction may be propagated among the magnet particles when the magnet particles tightly aggregate. As a result, magnetization reversal easily occurs in the magnet particles in a case where a magnetic field is applied from outside, causing the decrease of coercive force, which has been problematic.

Further, it would be practicable to add the grain growth inhibitor in a state of being distributed into an organic solvent, to a Nd-based magnet so as to concentrate the grain growth inhibitor in grain boundaries of the magnet. Generally speaking, however, once an organic solvent is added to a magnet, carbon-containing substances remain in the magnet even if the organic solvent is later volatilized by vacuum drying or the like. Since Nd and carbons exhibit significantly high reactivity therebetween, carbon-containing substances form carbide when remaining up to high-temperature stage in a sintering process. Consequently, the carbide thus formed makes a gap between a main phase and a grain boundary phase of the sintered magnet and accordingly the entirety of the magnet cannot be sintered densely, which causes a problem of serious degrade in the magnetic performance. Even if the gap is not made, the secondarily-formed carbide makes alpha iron separated out in the main phase of the sintered magnet, which causes a problem of serious degrade in the magnetic properties.

Further, addition of an organic solvent to magnet powder makes a grain growth inhibitor (e.g., refractory metal) present in a state being bound with oxygen contained in the organic solvent. Here, as Nd has high reactivity with oxygen, the presence of oxygen causes Nd to bind with the oxygen to form a Nd oxide at a sintering process. As a result, there occurs a problem of decrease of magnetic properties. Furthermore, binding of Nd with oxygen makes the Nd content deficient compared with the content based on the stoichiometric composition (Nd₂Fe₁₄B) . Consequently, alpha iron separates out in the main phase of the sintered magnet, which causes a problem of serious degrade in the magnetic properties. The problem becomes specifically significant in a case where extra Nd is not contained in the magnet raw material with respect to the stoichiometric composition.

Here, an HDDR process can be named as another method for obtaining highly refined magnet powder. However, the HDDR process has the same problem that the exchange interaction cannot be sufficiently disrupted among crystal grains.

The present invention has been made to resolve the above described conventional problem and the object thereof is to provide a manufacturing method for a permanent magnet capable of: inhibiting grain growth of magnet grains having single domain particle size during sintering; preventing magnetic reversal of each crystal grain by disrupting exchange interaction among crystal grain after sintering so as to achieve improvement of magnetic properties; previously reducing oxygen content contained in magnet particles by calcining the organometallic-compound-added magnet powder before sintering, specifically, calcination by plasma heating; and preventing degrade in the magnetic properties.

### MEANS FOR SOLVING THE PROBLEM

To achieve the above object, the present invention provides a permanent magnet manufactured through steps of: milling magnet material into magnet powder; adding an organometallic compound expressed with a structural formula of M-(OR)ₓ (M representing V, Mo, Zr, Ta, Ti, W or Nb, R representing a substituent group consisting of a straight-chain or branched-chain hydrocarbon, and ₓ representing an arbitrary integer) to the magnet powder obtained at the step of milling magnet material and getting the organometallic compound adhered to particle surfaces of the magnet powder; calcining the magnet powder of which particle surfaces have got adhesion of the organometallic compound by plasma heating so as to obtain a calcined body; compacting the calcined body so as to obtain a compact body; and sintering the compact body.

To achieve the above object, the present invention provides a manufacturing method of a permanent magnet comprising steps of: milling magnet material into magnet powder; adding an organometallic compound expressed with a structural formula of M-(OR)ₙ (M representing V, Mo, Zr, Ta, Ti, W or Nb, R representing a substituent group consisting of a straight-chain or branched-chain hydrocarbon, and ₙ representing the valence of metal or metalloid) to the magnet powder obtained at the step of milling magnet material and getting the organometallic compound adhered to particle surfaces of the magnet powder; characterized in that the manufacturing method further comprises steps of : calcining the magnet powder of which particle surfaces have got adhesion of the organometallic compound by plasma heating so as to obtain a calcined body in which metal oxides of M having been bound with O contained in the organometallic compound are reduced; compacting the calcined body so as to obtain a compact body; and sintering the compact body, wherein the permanent magnet is Nd-Fe-B based, and the permanent magnet includes Nd within a range of 25 through 37 wt%, Fe within a range of 60 through 75 wt% and B within a rage of 1 through 2 wt%.

To achieve the above object, the present invention further provides a manufacturing method of a permanent magnet comprising steps of: milling magnet material into magnet powder; adding an organometallic compound expressed with a structural formula of M- (OR)ₙ (M representing V, Mo, Zr, Ta, Ti, W or Nb, R representing a substituent group consisting of a straight-chain or branched-chain hydrocarbon, and ₙ representing the valence of metal or metalloid) to the magnet powder obtained at the step of milling magnet material and getting the organometallic compound adhered to particle surfaces of the magnet powder; compacting the magnet powder of which particle surfaces have got adhesion of the organometallic compound so as to obtain a compact body; characterized in that the manufacturing methodfurther comprises steps of: calcining the compact body by plasma heating so as to obtain a calcined body in which metal oxides of M having been bound with O contained in the organometallic compound are reduced; and sintering the calcined body, wherein the permanent magnet is Nd-Fe-B based, and the permanent magnet includes Nd within a range of 25 through 37 wt%, Fe within a range of 60 through 75 wt% and B within a range of 1 through 2 wt%.

In the above-described manufacturing method of a permanent magnet of the present invention, the calcined body is obtained at the step of calcining by high temperature hydrogen plasma heating.

In the above-described manufacturing method of a permanent magnet of the present invention, at the step of milling magnet material, the magnet material is milled into magnet powder so as to obtain magnet powder having single domain particle size.

In the above-described manufacturing method of a permanent magnet of the present invention, R in the structural formula is an alkyl group.

In the above-described manufacturing method of a permanent magnet of the present invention, R in the structural formula is an alkyl group of which carbon number is any one of integer numbers 2 through 6.

### EFFECT OF THE INVENTION

According to the manufacturing method of a permanent magnet of the present invention, it is made possible to manufacture a permanent magnet configured such that V, Mo, Zr, Ta, Ti, W, or Nb contained in the organometallic compound can be efficiently concentrated in grain boundaries of the magnet. As a result, in the manufactured permanent magnet, grain growth in the magnet particles at sintering can be inhibited and at the same, magnetization reversal of each crystal grain is prevented through disrupting exchange interaction among the crystal grains, enabling magnetic properties to be improved. Furthermore, as the additive amount of V, Mo, Zr, Ta, Ti, W, or Nb can be made smaller than that in a conventional method, the residual magnetic flux density can be inhibited from lowering. Furthermore, as the additive amount of V, Mo, Zr, Ta, Ti, W or Nb can be made smaller than that in a conventional method, the residual magnetic flux density can be inhibited from lowering. Furthermore, since the magnet powder to which the organometallic compound is added is calcined by plasma heating prior to sintering, oxygen content contained in magnet particles can be reduced before sintering of the magnet. Consequently, since such mannered manufacturing process can prevent alpha iron from separating out in a main phase of the sintered magnet and also prevent formation of oxides, serious degrade in the magnetic properties can be avoided.

Furthermore, the calcination process is performed to the powdered magnet particles, which is advantageous in that the reduction of metal oxides can be performed more easily to the whole magnet particles, compared with a case where the magnet particles are calcined after compaction. That is, the oxygen content in the powdered magnet particles can be more reliably decreased.

According to the manufacturing method of a permanent magnet of the present invention, it is made possible to manufacture a permanent magnet configured such that V, Mo, Zr, Ta, Ti, W, or Nb contained in the organometallic compound can be efficiently concentrated in grain boundaries of the magnet. As a result, in the manufactured permanent magnet, grain growth in the magnet particles at sintering can be inhibited and at the same, magnetization reversal of each crystal grain is prevented through disrupting exchange interaction among the crystal grains, enabling magnetic properties to be improved. Furthermore, as the additive amount of V, Mo, Zr, Ta, Ti, W, or Nb can be made smaller than that in a conventional method, the residual magnetic flux density can be inhibited from lowering. Furthermore, since the compact body consisting of organometallic-compound-added magnet powder is calcined by plasma heating prior to sintering, oxygen content contained in magnet particles can be reduced before sintering of the magnet. Consequently, since such mannered manufacturing process can prevent alpha iron from separating out in a main phase of the sintered magnet and also prevent formation of oxides, serious degrade in the magnetic properties can be avoided.

According to the manufacturing method of a permanent magnet of the present invention, since the high temperature hydrogen plasma heating is applied as specific means for calcination, high concentration of hydrogen radicals can be generated. Accordingly, even if the metal forming an organometallic compound is present in the magnet powder in a state of a stable oxide, the reduction to a metal or lowering of the oxidation number thereof can be easily performed at a low temperature using the hydrogen radicals.

According to the manufacturing method of a permanent magnet of the present invention, grain growth during sintering can be prohibited with respect to magnet particles having single domain particle size. Furthermore, through inhibiting the grain growth, the crystal grain of the sintered permanent magnet can be made to have a single domain structure. As a result, the magnetic property of the permanent magnet can be drastically improved.

According to the manufacturing method of a permanent magnet of the present invention, the organometallic compound composed of alkyl group is preferably used as organometallic compound to be added to the magnet powder. Therefore, thermal decomposition of the organometallic compound can be caused easily. Consequently, in a case where magnet powder or a compact body is calcined in hydrogen prior to sintering, for instance, carbon content in the magnet powder or the compact body can be reduced more reliably. Accordingly, such mannered manufacturing process can prevent alpha iron from separating out within the main phase of the sintered magnet. Thereby, the whole magnet can be densely sintered and the lowering of the coercive force can be prevented.

According to the manufacturing method of a permanent magnet of the present invention, the organometallic compound composed of alkyl group of carbon number 2-6 is preferably used as organometallic compound to be added to the magnet powder. Therefore, thermal decomposition of the organometallic compound can be caused at a low temperature. Consequently, in a case where magnet powder or a compact body is calcined in hydrogen prior to sintering, for instance, thermal decomposition of the organometallic compound can be easily caused to the whole magnet powder or the whole compact body. That is, through the calcination process, carbon content contained in the magnet powder or the compact body can be reduced more reliably.

### BRIEF DESCRIPTION OF THE DRAWINGS

[FIG. 1] is an overall view of a permanent magnet.
[FIG. 2] is an enlarged schematic view in vicinity of grain boundaries of the permanent magnet.
[FIG. 3] is an enlarged schematic view in vicinity of grain boundaries of the permanent magnet.
[FIG. 4] is a pattern diagram illustrating a magnetic domain structure of the permanent magnet.
[FIG. 5] is an explanatory diagram illustrating manufacturing processes of a permanent magnet according to a first manufacturing method of the invention.
[FIG. 6] is an explanatory diagram accounting for superiority of calcination process by high temperature hydrogen plasma heating.
[FIG. 7] is an explanatory diagram illustrating manufacturing processes of a permanent magnet according to a second manufacturing method of the invention.
[FIG. 8] is a chart depicting spectra detected in a range of 200 eV - 215 eV binding energy, with respect to a permanent magnet of an embodiment and a permanent magnet of a comparative example.
[FIG. 9] is a chart depicting a result on waveform analysis of the spectra of FIG. 8.

### BEST MODE FOR CARRYING OUT THE INVENTION

Specific embodiments of a method for manufacturing the permanent magnet according to the present invention will be described below in detail with reference to the drawings.

### [Constitution of Permanent Magnet]

First, a constitution of a permanent magnet 1 will be described. FIG. 1 is an overall view of the permanent magnet 1 produced according to the present invention. Incidentally, the permanent magnet 1 depicted in FIG. 1 is formed into a cylindrical shape. However, the shape of the permanent magnet 1 may be changed in accordance with the shape of a cavity used for compaction.

The permanent magnet 1 produced according to the present invention is an Nd-Fe-B-based magnet used. Further, Nb (niobium), V (vanadium), Mo (molybdenum), Zr (zirconium), Ta (tantalum), Ti (titanium) or W (tungsten) for increasing the coercive force of the permanent magnet 1 is concentrated on the boundary faces (grain boundaries) of Nd crystal grains forming the permanent magnet 1. Incidentally, the contents of respective components are regarded as Nd: 25 to 37 wt%, any one of Nb, V, Mo, Zr, Ta, Ti and W (hereinafter referred to as "Nb (or other) ") : 0.01 to 5 wt%, B: 1 to 2 wt%, and Fe (electrolytic iron): 60 to 75 wt%. Furthermore, the permanent magnet 1 may include other elements such as Co, Cu, Al or Si in small amount, in order to improve the magnetic properties thereof.

Specifically, in the permanent magnet 1 according to the present invention, Nb (or other) is concentrated onto the grain boundaries of the Nd crystal grains 10 by generating a layer 11 (hereinafter referred to as refractory metal layer 11) in which Nb (or other) being a refractory metal substitutes for part of Nd on each surface (outer shell) of the Nd crystal grains 10 constituting the permanent magnet 1 as depicted in FIG. 2. FIG. 2 is an enlarged view showing the Nd crystal grains 10 constituting the permanent magnet 1. The refractory metal layer 11 is preferably nonmagnetic.

Here, in the present invention, the substitution of Nb (or other) is carried out before compaction of magnet powder through addition of an organometallic compound containing Nb (or other) milled as later described. Specifically, here, the organometallic compound containing the Nb (or other) is uniformly adhered to the particle surfaces of the Nd crystal grains 10 by wet dispersion and the Nb (or other) included in the organometallic compound diffusively intrudes into the crystal growth region of the Nd crystal grains 10 and substitutes for Nd, to form the refractory metal layers 11 shown in FIG. 2, when the magnet powder to which the organometallic compound containing Nb (or other) is added is sintered. Incidentally, the Nd crystal grain 10 may be composed of, for example, Nd₂Fe₁₄B intermetallic compound, and the refractory metal layer 11 may be composed of, for example, NbFeB intermetallic compound.

Furthermore, in the present invention, specifically as later described, the organometallic compound containing Nb (or other) is expressed by M- (OR)ₙ (in the formula, M represents V, Mo, Zr, Ta, Ti, W or Nb, R represents a substituent group consisting of a straight-chain or branched-chain hydrocarbon and ₙ represents the valence of metal or metalloid), and the organometallic compound containing Nb (or other) (such as niobium ethoxide, niobium n-propoxide, niobium n-butoxide, niobium n-hexoxide) is added to an organic solvent and in a wet condition, mixed with the magnet powder. Thus, the organometallic compound containing Nb (or other) is dispersed in the organic solvent, enabling the organometallic compound containing Nb (or other) to be adhered onto the particle surfaces of Nd crystal grains 10 effectively.

The metal alkoxide is expressed by a general formula M-(OR)ₙ (M: metal element, R: organic group, n: valence of metal or metalloid). Furthermore, examples of metal or metalloid composing the metal alkoxide include W, Mo, V, Nb, Ta, Ti, Zr, Ir, Fe, Co, Ni, Cu, Zn, Cd, Al, Ga, In, Ge, Sb, Y, lanthanide and the like. However, in the present invention, refractory metal is specifically used. Furthermore, for the purpose of preventing interdiffusion with the main phase of the magnet at sintering to be later described, V, Mo, Zr, Ta, Ti, W or Nb is used from among refractory metals.

Furthermore, the types of the alkoxide are not specifically limited, and there may be used, for instance, methoxide, ethoxide, propoxide, isopropoxide, butoxide or alkoxide carbon number of which is 4 or larger. However, in the present invention, those of low-molecule weight are used in order to inhibit the carbon residue by means of thermal decomposition at a low temperature to be later described. Furthermore, methoxide carbon number of which is 1 is prone to decompose and difficult to deal with, therefore it is preferable to use alkoxide carbon number of which is 2 through 6 included in R, such as ethoxide, isopropoxide, propoxide or butoxide. That is, in the present invention, it is preferable to use, as the organometallic compound to be added to the magnet powder, an organometallic compound expressed by M- (OR)ₙ (in the formula, M represents V, Mo, Zr, Ta, Ti, W or Nb, R represents a straight-chain or branched-chain alkyl group and ₙ represents the valence of metal or metalloid) or it is more preferable to use an organometallic compound expressed by M-(OR)ₙ (in the formula, M represents V, Mo, Zr, Ta, Ti, W or Nb, R represents a straight-chain or branched-chain alkyl group of which carbon number is 2 through 6, and ₙ represents the valence of metal or metalloid).

Furthermore, a compact body compacted through powder compaction can be sintered under appropriate sintering conditions so that Nb (or other) can be prevented from being diffused or penetrated (solid-solutionized) into the Nd crystal grains 10. Thus, in the present invention, even if Nb (or other) is added, Nb (or other) can be concentrated only within the grain boundaries after sintering. As a result, the phase of the Nd₂Fe₁₄B intermetallic compound of the core accounts for the large proportion in volume, with respect to crystal grains as a whole (in other words, the sintered magnet in its entirety) . Accordingly, the decrease of the residual magnetic flux density (magnetic flux density at the time when the intensity of the external magnetic field is brought to zero) can be inhibited.

Further, generally, in a case where sintered Nd crystal grains 10 are densely aggregated, exchange interaction is presumably propagated among the Nd crystal grains 10. As a result, when a magnetic field is applied from outside, magnetization reversal easily takes place in the crystal grains, and coercive force thereof decreases even if sintered crystal grains can be made to have a single domain structure. However, in the present invention, there are provided refractory metal layers 11 which are nonmagnetic and coat the surfaces of the Nd crystal grains 10, and the refractory metal layers 11 disrupt the exchange interaction among the Nd crystal grains 10. Accordingly, magnetization reversal can be prevented in the crystal grains, even if a magnetic field is applied from outside.

Furthermore, the refractory metal layers 11 coating the surfaces of the Nd crystal grains 10 operate as means of inhibiting what-is-called grain growth in which an average particle diameter increases in Nd crystal grains 10 at the sintering of the permanent magnet 1. Hereinafter, the mechanism of the inhibition of the grain growth in the permanent magnet 1 by the refractory metal layers 11 will be discussed referring to FIG. 3. FIG. 3 is a schematic view illustrating a magnetic domain structure of a ferromagnetic body.

Generally, there is excessive energy in a grain boundary which is an inconsistent interfacial boundary left between a crystal and another crystal. As a result, at high temperature, grain boundary migration occurs in order to lower the energy. Accordingly, when the magnet raw material is sintered at high temperature (for instance, 800 through 1150 degrees Celsius for Nd-Fe-B-based magnets), small magnet particles shrink and disappear, and remaining magnet particles grow in average diameter, in other words, what-is-called grain growth occurs.

Here, in the present invention, through adding the organometallic compound expressed by formula M-(OR)ₙ (in the formula, M represents V, Mo, Zr, Ta, Ti, W or Nb, R represents a substituent group consisting of a straight-chain or branched-chain hydrocarbon and ₙ represents the valence of metal or metalloid), Nb (or other), the refractory metal, is concentrated on the surfaces of the interfacial boundary of magnet particles as illustrated in FIG. 3. Then, due to the concentrated refractory metal, the grain boundary migration which easily occurs at high temperature can be prevented, and grain growth can be inhibited.

Furthermore, if an organometallic compound is added to the magnet powder, Nb (or other) is present in a state being bound with oxygen contained in the organometallic compound (such as NbO, Nb₂O₃, NbO₂ and Nb₂O₅). Here, as Nd has high reactivity with oxygen, the presence of oxygen causes Nd to bind with the oxygen to form a Nd oxide at a sintering process. As a result, there occurs a problem of decrease of magnetic properties. Furthermore, binding of Nd with oxygen makes the Nd content deficient compared with the content based on the stoichiometric composition (Nd₂Fe₁₄B). Consequently, alpha iron separates out in the main phase of the sintered magnet, which causes a problem of serious degrade in the magnetic properties. Especially, the problem is serious in a case where Nd is included in magnet raw material with less quantity in comparison with Nd included in the stoichiometric composition. However, Nb (or other) present in the state being bound with oxygen can be reduced to metal Nb (or other) or to oxides with smaller oxidation number (namely, to lower the oxidation number) through calcination process by later-described plasma heating. Thus, the oxygen therein can be lowered. As a result, such mannered manufacturing process can prevent binding of oxygen with Nd at the sintering process and also prevent alpha iron from separating out.

Furthermore, it is desirable that the particle diameter D of the Nd crystal grain 10 is from 0.2µm to 1.2µm, preferably approximately 0.3µm. Also, it is desirable that thickness d of the refractory metal layers 11 is from 1 nm to 200 nm, preferably, 2 nm to 50 nm. The above specified range for the thickness d of the refractory metal layers 11 is enough to prevent the grain growth of the Nd magnet particles during sintering, and to disrupt exchange interaction among the Nd crystal grains 10. However, if the thickness d of the refractory metal layers 11 excessively increases, the rate of nonmagnetic components which exert no magnetic properties becomes large, so that the residual magnet flux density becomes low.

Then, it becomes possible to make the Nd crystal grain 10 have a single domain structure if the grain size d of the Nd crystal grain 10 is set to be approximately 0.2 µm to 1.2 µm, or preferably approximately 0.3 µm. Consequently, the magnetic property of the permanent magnet 1 can be drastically improved.

However, as a configuration for concentrating refractory metal on the grain boundaries of the Nd crystal grains 10, there may be employed, as illustrated in FIG. 4, a configuration in which agglomerates 12 composed of refractory metal are scattered onto the grain boundaries of the Nd crystal grains 10. The similar effect (such as inhibiting grain growth and disrupting exchange interaction) can be obtained even in such a configuration as illustrated in FIG. 4. The concentration of refractory metal in the grain boundaries of the Nd crystal grains 10 can be confirmed, for instance, through scanning electron microscopy (SEM), transmission electron microscopy (TEM) or three-dimensional atom probe technique.

Incidentally, the refractory metal layer 11 is not required to be a layer composed of only one of Nb compound, V compound, Mo compound, Zr compound, Ta compound, Ti compound and W compound (hereinafter referred to as "Nb compound (or other)"), and may be a layer composed of a mixture of a Nb compound (or other) and a Nd compound. In such a case, a layer composed of the mixture of the Nb compound (or other) and the Nd compound are formed by adding the Nd compound. As a result, the liquid-phase sintering of the Nd magnet powder can be promoted at the time of sintering. The desirable Nd compound to be added may be NdH₂, neodymium acetate hydrate, neodymium(III) acetylacetonate trihydrate, neodymium(III) 2-ethylhexanoate, neodymium(III) hexafluoroacetylacetonate dihydrate, neodymium isopropoxide, neodymium(III) phosphate n-hydrate, neodymium trifluoroacetylacetonate, and neodymium trifluoromethanesulfonate or the like.

### [First Method for Manufacturing Permanent Magnet]

Next, the first method for manufacturing the permanent magnet 1 directed to the present invention will be described below with reference to FIG. 5. FIG. 5 is an explanatory view illustrating a manufacturing process in the first method for manufacturing the permanent magnet 1 directed to the present invention.

First, there is manufactured an ingot comprising Nd-Fe-B of certain fractions (for instance, Nd: 32.7 wt%, Fe (electrolytic iron) : 65.96 wt%, and B: 1.34 wt%). Thereafter the ingot is coarsely milled using a stamp mill, a crusher, etc. to a size of approximately 200 µm. Otherwise, the ingot is dissolved, formed into flakes using a strip-casting method, and then coarsely powdered using a hydrogen pulverization method.

Next, the coarsely milled magnet powder is finely milled with a jet mill 41 to form fine powder of which the average particle diameter is smaller than a predetermined size (for instance, 0.1 µm through 5.0 µm), more preferably ultrafine powder having an average particle size of single domain particle size(for instance, 0.2 µm through 1.2 µm), in: (a) an atmosphere composed of inert gas such as nitrogen gas, argon (Ar) gas, helium (He) gas or the like having an oxygen content of substantially 0 %; or (b) an atmosphere composed of inert gas such as nitrogen gas, Ar gas, He gas or the like having an oxygen content of 0.0001 through 0.5 %. Here, the term "having an oxygen content of substantially 0 %" is not limited to a case where the oxygen content is completely 0 %, but may include a case where oxygen is contained in such an amount as to allow a slight formation of an oxide film on the surface of the fine powder. Furthermore, ultrafine powder having an average particle size of the single domain particle size may be composed mostly of magnet particles of single domain structure, and furthermore, may include magnet particles other than those having the average particle size.

In the meantime, organometallic compound solution is prepared for adding to the fine powder finely milled by the jet mill 41. Here, an organometallic compound containing Nb (or other) is added in advance to the organometallic compound solution and dissolved therein. Incidentally, in the present invention, it is preferable to use, as the organometallic compound to be dissolved, an organometallic compound (such as niobium ethoxide, niobium n-propoxide, niobium n-butoxide or niobium n-hexoxide) pertinent to formula M- (OR)ₙ (in the formula, M represents V, Mo, Zr, Ta, Ti, W or Nb, R represents a straight-chain or branched-chain alkyl group of which carbon number is 2 through 6 and ₙ represents the valence of metal or metalloid). Furthermore, the amount of the organometallic compound containing Nb (or other) to be dissolved is not particularly limited, however, it is preferably adjusted to such an amount that the Nb (or other) content with respect to the sintered magnet is 0.001 wt% through 10 wt%, or more preferably, 0.01 wt% through 5 wt%, as above described.

Successively, the above organometallic compound solution is added to the fine powder classified with the jet mill 41. Through this, slurry 42 in which the fine powder of magnet raw material and the organometallic compound solution are mixed is prepared. Here, the addition of the organometallic compound solution is performed in an atmosphere composed of inert gas such as nitrogen gas, Ar gas or He gas.

Thereafter, the prepared slurry 42 is desiccated in advance through vacuum desiccation or the like before compaction and desiccated magnet powder 43 is obtained. Thereafter, the desiccated magnet powder 43 undergoes a calcination process by plasma heating with high temperature hydrogen plasma. Specifically, the calcination process is performed by putting the magnet powder 43 into a plasma heating apparatus that utilizes "2.45 GHz high-frequency microwaves". To be more specific, in the apparatus, application of voltage to the mixed gas of hydrogen gas and inert gas (for example, Ar gas) causes plasma excitation so as to irradiate the thus generated high temperature hydrogen plasma on the magnet powder 43 for calcination. Incidentally, the flow rate for the supplied gas is within a range of 1 L/min - 10 L/min for hydrogen flow and 1 L/min - 5 L/min for Argon flow. The output voltage at plasma excitation is within a range of 1 kW - 10 kW, and the plasma-irradiation period is within a range of 1-60 seconds.

In the above calcination process by the plasma heating, it becomes possible to reduce metal oxides which are present in a state being bound with oxygen (such as NbO, Nb₂O₃, NbO₂ and Nb₂O₅) to metal Nb (or other), or to perform reduction to oxides with smaller oxidation number (namely, to lower the oxidation number) such as NbO and the like, thereby decreasing in advance the oxygen contained in the magnet powder. As a result, a Nb oxide or the like contained in the magnet powder is reduced before sintering, and the oxygen contained in the magnet powder can be decreased in advance. As a result, in the later sintering process, there does not occur the binding of Nd and oxygen or the formation of Nd oxides, and also alpha iron can be prevented from separating out. Furthermore, specifically in the calcination utilizing the high temperature hydrogen plasma heating, hydrogen radicals can be generated. Using the hydrogen radicals, it becomes possible to perform the reduction to metal Nb (or other) or to easily lower the oxidation number in low temperature. Compared with a case of using low temperature hydrogen plasma, the concentration of hydrogen radicals can be made higher in a case of using high temperature hydrogen plasma. Accordingly, stable metal oxides (such as Nb₂O₅ and the like) having low free energy of formation can be appropriately reduced.

Hereinafter, the superiority of the calcination process using plasma heating is discussed in more detail referring to FIG. 6.

For reducing the stable metal oxides with low free energy of formation (such as Nb₂O₅) to metal, it generally requires strong reduction means such as (1) calcium reduction, (2) fused salt electrolysis, (3) laser reduction and the like. However, with such a strong reduction method, the object to be reduced is heated to very high temperature. Therefore, if such a method is performed to Nd magnet particles like those in the present invention, there is a risk that the Nd magnet particles may be fused.

Here, as has been discussed above, the calcination by the above high temperature hydrogen plasma heating makes it possible to form hydrogen radicals in high concentration. Further, as illustrated in FIG. 6, the lower the temperature is, the stronger reducing character is shown in the reduction by hydrogen radicals. Accordingly, even the stable metal oxide with low free energy of formation such as Nb₂O₅ can be reduced in lower temperature than that in the above-mentioned reduction methods (1)-(3). Incidentally, practicability of low temperature reduction may be indicated by the fact that the sintered Nd magnet particles are not fused.

Furthermore, in addition to the above calcination process by the above plasma and the like, another calcination process (calcination process in hydrogen) may be held for several hours (five hours, for instance) in hydrogen atmosphere at 200 through 900 degrees Celsius, more preferably, 400 through 900 degrees Celsius. The timing to perform the calcination process in hydrogen may be either before or after the calcination process by the above plasma heating. Furthermore, the calcination process may be performed to magnet powder either before or after the compaction. During the calcination process in hydrogen, so-called decarbonization is performed in such a manner that carbon content in the calcined body is lowered by causing thermal decomposition to the organometallic compound. Furthermore, the calcination process in hydrogen is to be performed under a condition of less than 0.15 wt% carbon content in the calcined body, or more preferably less than 0.1 wt%. Accordingly, the permanent magnet 1 as a whole can be densely sintered in the following sintering process, and the decrease in the residual magnetic flux density and coercive force can be prevented. Furthermore, in a case where the calcination process in hydrogen is performed, a decarbonization process may be performed after the calcination process in order to lower the activity level of the calcined body activated through the calcination process in hydrogen. More specifically, the decarbonization process may be performed by holding the calcined body for 1-3 hours in vacuum atmosphere at 200 through 600 degrees Celsius, more preferably, 400 through 600 degrees Celsius. However, in a case where the sintering is performed without any exposure to the external air after calcination in hydrogen, the dehydrogenation process becomes unnecessary.

Next, the powdered calcined body 65 calcined at the calcination process by the plasma heating is powder-compacted into a predetermined shape by the compaction device 50.

As illustrated in FIG. 5, the compaction device 50 has a cylindrical mold 51, a lower punch 52 and an upper punch 53, and a space surrounded therewith forms a cavity 54.

In the compaction device 50, a pair of magnetic field generating coils 55 and 56 are disposed in the upper and lower positions of the cavity 54 so as to apply magnetic flux to the calcined body 65 filling the cavity 54. The magnetic field to be applied may be, for instance, 795.9 kA·m⁻¹ (10 kOe).

When performing the powder compaction, firstly, the cavity 54 is filled with the calcined body 65. Thereafter, the lower punch 52 and the upper punch 53 are activated to apply pressure against the calcined body 65 filling the cavity 54 in a pressurizing direction of arrow 61, thereby performing compaction thereof. Furthermore, simultaneously with the pressurization, pulsed magnetic field is applied to the calcined body 65 filling the cavity 54, using the magnetic field generating coils 55 and 56, in a direction of arrow 62 which is parallel with the pressuring direction. As a result, the magnetic field is oriented in a desired direction. Incidentally, it is necessary to determine the direction in which the magnetic field is oriented while taking into consideration the magnetic field orientation required for the permanent magnet 1 formed from the calcined body 65.

After that, there is performed a sintering process for sintering the compacted-state calcined body 65. However, as a sintering method for a compact body, there can be employed, besides commonly-used vacuum sintering, pressure sintering in which the compact body is sintered in a pressured state. For instance, when the sintering is performed in the vacuum sintering, the temperature is risen to approximately 800 through 1080 degrees Celsius in a given rate of temperature increase and held for approximately two hours. During this period, the vacuum sintering is performed, and the degree of vacuum is preferably equal to or smaller than 10⁻⁴ Torr. The compact body is then cooled down, and again undergoes a heat treatment in 600 through 1000 degrees Celsius for two hours. As a result of the sintering, the permanent magnet 1 is manufactured.

Meanwhile, the pressure sintering includes, for instance, hot pressing, hot isostatic pressing (HIP), spark plasma sintering (SPS) and the like. However, it is preferable to adopt the spark plasma sintering which is uniaxial pressure sintering in which pressure is uniaxially applied and also in which sintering is performed by electric current sintering, so as to prevent grain growth of the magnet particles during the sintering and also to prevent warpage formed in the sintered magnets. Incidentally, the following are the preferable conditions when the sintering is performed in the SPS; pressure is applied at 30 MPa, the temperature is risen in a rate of 10 degrees Celsius per minute until reaching 940 degrees Celsius in vacuum atmosphere of several Pa or lower and then the state of 940 degrees Celsius in vacuum atmosphere is held for approximately five minutes. The compact body is then cooled down, and again undergoes a heat treatment in 600 through 1000 degrees Celsius for two hours. As a result of the sintering, the permanent magnet 1 is manufactured.

### [Second Method for Manufacturing Permanent Magnet]

Next, the second method for the manufacturing the permanent magnet 1 which is an alternative manufacturing method will be described below with reference to FIG. 7. FIG. 7 is an explanatory view illustrating a manufacturing process in the second method for manufacturing the permanent magnet 1 directed to the present invention.

The process until the slurry 42 is manufactured is the same as the manufacturing process in the first manufacturing method already discussed referring to FIG. 5, therefore detailed explanation thereof is omitted.

First, the prepared slurry 42 is desiccated in advance through vacuum desiccation or the like before compaction and desiccated magnet powder 43 is obtained. Then, the desiccated magnet powder is subjected to powder-compaction to form a given shape using a compaction device 50. There are dry and wet methods for the powder compaction, and the dry method includes filling a cavity with the desiccated fine powder and the wet method includes preparing slurry of the desiccated fine powder using solvent and then filling a cavity therewith. In this embodiment, a case where the dry method is used is described as an example. Furthermore, the organometallic compound solution can be volatilized at the sintering stage after compaction. Incidentally, details of the compaction device 50 are omitted because manufacturing processes performed here in the second method are the same as those of the first method already described by referring to FIG. 5. Furthermore, in a case where the wet method is used, slurry may be injected while applying the magnetic field to the cavity 54, and in the course of the injection or after termination of the injection, a magnetic field stronger than the initial magnetic field may be applied to perform the wet molding. Furthermore, the magnetic field generating coils 55 and 56 may be disposed so that the application direction of the magnetic field is perpendicular to the pressuring direction.

Thereafter, the compact body 71 obtained through powder-compaction undergoes a calcination process by plasma heating with high temperature hydrogen plasma. Specifically, the calcination process is performed by putting the compact body 71 into a plasma heating apparatus. To be more specific, in the apparatus, application of voltage to the mixed gas of hydrogen gas and inert gas (for example, Ar gas) causes plasma excitation so as to irradiate the thus generated high temperature hydrogen plasma on the compact body 71 for calcination. Incidentally, the flow rate for the supplied gas is within a range of 1 L/min - 10 L/min for hydrogen flow and 1 L/min - 5 L/min for Argon flow. The output voltage at plasma excitation is within a range of 1 kW - 10 kW, and the plasma-irradiation period is within a range of 1-60 seconds.

Then, there is performed a sintering process for sintering the compact body 71 calcined through plasma heating. The sintering process is performed by the vacuum sintering or the pressure sintering similar to the above first manufacturing method. Details of the sintering condition are omitted because the manufacturing process here is similar to that of the first manufacturing method already described. As a result of the sintering, the permanent magnet 1 is manufactured.

The first manufacturing method discussed above has an advantage that the calcination process in hydrogen is performed to the powdery magnet particles, reduction of metal oxides can be performed to the whole magnet particles in comparison with the second manufacturing method in which the calcination process is performed to the compacted magnet particles. That is, the first manufacturing method makes it possible to more securely decrease the oxygen content in the calcined body, in comparison with the second manufacturing method.

### [Embodiment]

Here will be described an embodiment according to the present invention referring to a comparative example for comparison.

### (Embodiment)

In comparison with fraction regarding alloy composition of a neodymium magnet according to the stoichiometric composition (Nd: 26.7 wt%, Fe (electrolytic iron): 72.3 wt%, B: 1.0 wt%), proportion of Nd in that of the neodymium magnet powder for the embodiment 1 is set higher, such as Nd/ Fe/ B= 32.7/ 65.96/ 1.34 in wt%, for instance. Further, 5 wt% of niobium n-propoxide has been added as organometallic compound to milled neodymium magnet powder. A calcination process with plasma heating has been performed by using high temperature hydrogen plasma. Regarding flow rate of gases to be supplied during the calcination process, both hydrogen feed rate and Argon feed rate are set to 3 L/min. The output voltage at plasma excitation is set to 3 kW, and the plasma-irradiation is performed for 60 seconds. Sintering of the compacted-state calcined body has been performed in the SPS. Other processes are the same as the processes in [First Method for Manufacturing Permanent Magnet] mentioned above.

### (Comparative Example)

Niobium n-propoxide has been used as organometallic compound to be added, and sintering has been performed without undergoing a calcination process by plasma heating. Other conditions are the same as the conditions in the embodiment.

### (Comparative Analysis on Embodiment and Comparative Example in View of Application/Non-application of Calcination Process by Plasma Heating)

Permanent magnets according to the embodiment and the comparative example are analyzed using an X-ray photoelectron spectrometer (or electron spectrometer for chemical analysis, ESCA) . FIG. 8 is a chart depicting spectra detected in a range of 200 eV - 215 eV binding energy, with respect to the permanent magnets of the embodiment and the comparative example. FIG. 9 is a chart depicting a result of waveform analysis of the spectra of FIG. 8.

AS illustrated in FIG. 8, the permanent magnets of the embodiment and the comparative example have different spectral shapes with each other. Here, the mixture proportion with respect to each spectrum is calculated based on the standard sample, and the proportions of Nb, NbO, Nb₂O₃, NbO₂ and Nb₂O₅ are depicted respectively in FIG. 9. As shown in FIG. 9, Nb comprises 81% and NbO, an Nb oxide, comprises 19% in the permanent magnet of the embodiment, whereas Nb comprises nearly 0% and Nb₂O₅, an Nb oxide, comprises nearly 100% in the permanent magnet of the comparative example.

That is, with respect to the permanent magnet according to the embodiment after the calcination process by plasma heating, most part of Nb oxides (NbO, Nb₂O₃, NbO₂ and Nb₂O₅) which have been present in the state bound with oxygen is successfully reduced to metal Nb. Even if the reduction of Nb oxides may not reach the metal Nb state, the Nb oxides can still be reduced to oxides with smaller oxidation number (in other words, the oxidation number can be lowered) such as NbO, so that the oxygen contained in the magnet powder can be decreased in advance. Thus, in the permanent magnet of the embodiment, the Nb oxide or the like contained in the magnet powder can be reduced before sintering, so that the oxygen contained in the magnet powder can be reduced in advance. Thereby, the binding of Nd and oxygen and the formation of a Nd oxide in the later sintering process can be prevented. Accordingly, in the permanent magnet of the embodiment, deterioration of the magnet properties due to presence of the metal oxides can be prevented and alpha iron can be prevented from separating out. That is, a permanent magnet with high quality can be obtained.

Meanwhile, the permanent magnet of the comparative example has a large proportion of remnant Nb oxides, therefore Nd is likely to bind with oxygen in the sintering process, and Nd oxides are formed. Further, alpha iron separates out in large amount. As a result, deterioration of the magnetic properties occurs in the comparative example.

As described in the above, with respect to the permanent magnet 1 and the manufacturing method of the permanent magnet 1 directed to the above embodiment, an organometallic compound solution is added to fine powder of milled neodymium magnet so as to uniformly adhere the organometallic compound to particle surfaces of the neodymium magnet powder, the organometallic compound being expressed with a structural formula of M-(OR)ₓ (M represents V, Mo, Zr, Ta, Ti, W or Nb, R represents a substituent group consisting of a straight-chain or branched-chain hydrocarbon and x represents an arbitrary integer). After that, the magnet powder is calcined by plasma heating. Thereafter, a compact body formed through powder compaction undergoes vacuum sintering or pressure sintering, whereby the permanent magnet is manufactured. Owing to the above processes, even though amount of to-be-added Nb (or other) is made less in comparison with conventional one, Nb (or other) added thereto can be efficiently concentrated in grain boundaries of the magnet. Consequently, grain growth can be prevented in the magnet particles at sintering, and at the same time exchange interaction can be disrupted among the magnet particles after sintering so as to prevent magnetization reversal in the magnet particles, making it possible to improve the magnetic performance thereof. Further, decarbonization is made easier when adding the above specified organometallic compound to magnet powder in comparison with when adding other organometallic compounds. Furthermore, such sufficient decarbonization can avoid decline in coercive force which is likely to be caused by carbon contained in the sintered magnet. Furthermore, owing to such sufficient decarbonization, the entirety of the magnet can be sintered densely.

Still further, Nb (or other) being refractory metal is concentrated in grain boundaries of the sintered magnet. Therefore, Nb (or other) concentrated in the grain boundaries inhibits grain growth in the magnet particles at sintering and, and at the same time, disrupts exchange interaction among the magnet particles after sintering so as to prevent magnetization reversal in the magnet particles, making it possible to improve the magnetic performance thereof. Further, since amount of Nb (or other) added thereto is less in comparison with conventional amount thereof, decline in residual magnetic flux density can be avoided.

Furthermore, Nb (or other) concentrated in the grain boundaries of a magnet forms a layer of 1 nm - 200 nm, preferably 2 nm - 50 nm in thickness on the surface of each magnet particle after sintering. Thereby, grain growth can be prevented in the magnet particles at sintering, and at the same time exchange interaction can be disrupted among the crystal grains after sintering so as to prevent magnetization reversal in the crystal grains, making it possible to improve the magnetic performance thereof.

Furthermore, the magnet raw material is finely pulverized into the magnet powder so as to include some magnet powder having single domain particle size. Thereby, grain growth of the magnet powder having single domain particle size can be inhibited at sintering. Furthermore, inhibition of the grain growth makes it possible to shape the crystal grain of the sintered magnet in a single domain structure. As a result, the magnetic property of the permanent magnet 1 can be drastically improved.

Further, the organometallic-compound-added magnet powder or the compact body is calcined by utilizing plasma heating prior to sintering. Thereby, such mannered manufacturing process makes it possible to reduce Nb (or other) present therein in a state bound with oxygen to metal Nb (or other), or to an oxide with smaller oxidation number such as NbO, etc. (that is, to lower the oxidation number) before sintering. Thus, even if the organometallic compound is added, there can be prevented the increase of the oxygen content contained in the magnet particles. Since such mannered manufacturing process prevents alpha iron from separating out in a main phase of the sintered magnet and also prevents formation of oxides, serious degrade in the magnetic properties can be avoided.

Furthermore, as the calcination process by plasma heating is performed under 1 kW - 10 kW output voltage, with 1 L/min - 10 L/min hydrogen flow and 1 L/min - 5 L/min Argon flow and for an irradiation time period of 1-60 seconds, the magnet powder or compact body can be calcined under an appropriate condition using plasma heating, so that the oxygen content contained in the magnet particle can be more reliably decreased. Moreover, as the high temperature hydrogen plasma heating is applied as specific means for calcination, high concentration of hydrogen radicals can be generated. Accordingly, even if the metal forming an organometallic compound is present in the magnet powder in a state of a stable oxide, the reduction to a metal or lowering of the oxidation number thereof can be easily performed at a low temperature using the hydrogen radicals.

Furthermore, specifically in the first manufacturing method, the calcination process is performed to the powdered magnet particles, which is advantageous in that the reduction of metal oxides can be performed more easily to the whole magnet particles, compared with the case where the magnet particles are calcined after compaction. That is, compared with the second manufacturing method, the oxygen content in the calcined body can be more reliably decreased.

Furthermore, if the organometallic compound to be added is specifically chosen from the organometallic compound composed of alkyl group, or more preferably an organometallic compound composed of alkyl group of carbon number 2-6, thermal decomposition of the organometallic compound can be caused at a low temperature when the magnet powder or the compact body is calcined in hydrogen atmosphere. Thereby, thermal decomposition of the organometallic compound can easily be caused to the whole magnet powder or the whole compact body. Accordingly, such mannered manufacturing process can prevent alpha iron from separating out within the main phase of the magnet after sintering. Thereby, the whole magnet can be densely sintered and the lowering of the coercive force can be prevented.

Not to mention, of magnet powder, milling condition, mixing condition, calcination condition, dehydrogenation condition, sintering condition, etc. are not restricted to conditions described in the embodiments.

Further, in the embodiment, niobium n-propoxide is used as organometallic compound to be added to magnet powder. Other organometallic compounds may be used as long as being an organometallic compound that satisfies a formula of M-(OR)ₙ (M represents V, Mo, Zr, Ta, Ti, W or Nb, R represents a substituent group consisting of a straight-chain or branched-chain hydrocarbon, and ₙ represents (the valence of metal or metalloid). For instance, there may be used an organometallic compound of which carbon number is 7 or larger and an organometallic compound including a substituent group consisting of carbon hydride other than an alkyl group.

### EXPLANATION OF REFERENCES

- 1: permanent magnet
- 10: Nd crystal grain
- 11: refractory metal layer
- 12: refractory metal agglomerate
- 42: slurry
- 43: magnet powder
- 65: calcined body
- 71: compact body

## Claims

1. A manufacturing method of a permanent magnet comprising steps of:
milling magnet material into magnet powder;
adding an organometallic compound expressed with a structural formula of
M-(OR)ₙ
M representing V, Mo, Zr, Ta, Ti, W or Nb, R representing a substituent group consisting of a straight-chain or branched-chain hydrocarbon, and ₙ representing the valence of metal or metalloid;
to the magnet powder obtained at the step of milling magnet material and getting the organometallic compound adhered to particle surfaces of the magnet powder;
**characterized in that** the manufacturing method further comprises steps of:
calcining the magnet powder of which particle surfaces have got adhesion of the organometallic compound by plasma heating so as to obtain a calcined body in which metal oxides of M having been bound with 0 contained in the organometallic compound are reduced;
compacting the calcined body so as to obtain a compact body; and
sintering the compact body,
wherein the permanent magnet is Nd-Fe-B based, and
the permanent magnet includes Nd within a range of 25 through 37 wt%, Fe within a range of 60 through 75 wt% and B within a range of 1 through 2 wt%.

2. A manufacturing method of a permanent magnet comprising steps of:
milling magnet material into magnet powder;
adding an organometallic compound expressed with a structural formula of
M-(OR)ₙ
M representing V, Mo, Zr, Ta, Ti, W or Nb, R representing a substituent group consisting of a straight-chain or branched-chain hydrocarbon, and ₙ representing the valence of metal or metalloid;
to the magnet powder obtained at the step of milling magnet material and getting the organometallic compound adhered to particle surfaces of the magnet powder;
compacting the magnet powder of which particle surfaces have got adhesion of the organometallic compound so as to obtain a compact body;
**characterized in that** the manufacturing method further comprises steps of:
calcining the compact body by plasma heating so as to obtain a calcined body in which metal oxides of M having been bound with O contained in the organometallic compound are reduced; and
sintering the calcined body,
wherein the permanent magnet is Nd-Fe-B based, and
the permanent magnet includes Nd within a range of 25 through 37 wt%, Fe within a range of 60 through 75 wt% and B within a range of 1 through 2 wt%.

3. The manufacturing method of a permanent magnet according to claim 1 or 2, wherein the calcined body is obtained at the step of calcining by high temperature hydrogen plasma heating.

4. The manufacturing method of a permanent magnet according to any of claims 1 through 3, wherein, at the step of milling magnet material, the magnet material is milled into magnet powder so as to obtain magnet powder having single domain particle size.

5. The manufacturing method of a permanent magnet according to any of claims 1 through 4, wherein R in the structural formula is an alkyl group.

6. The manufacturing method of a permanent magnet according to claim 5, wherein R in the structural formula is an alkyl group of which carbon number is any one of integer numbers 2 through 6.

## Patentansprüche

1. Herstellungsverfahren für einen Permanentmagneten, umfassend folgende Schritte:
Mahlen von Magnetmaterial zu Magnetpulver;
Zugeben einer metallorganischen Verbindung, ausgedrückt durch eine Strukturformel
M-(OR)ₙ
wobei M V, Mo, Zr, Ta, Ti, W oder Nb darstellt, R eine Substituentengruppe darstellt, die aus einem geradkettigen oder verzweigtkettigen Kohlenwasserstoff besteht, und n die Wertigkeit des Metalls oder Metalloids darstellt;
zu dem Magnetpulver, das bei dem Mahlschritt von Magnetmaterial erhalten wurde, und Anhaftenlassen der metallorganischen Verbindung an Teilchenoberflächen des Magnetpulvers;
**dadurch gekennzeichnet, dass** das Herstellungsverfahren ferner folgende Schritte umfasst:
Kalzinieren des Magnetpulvers, an dessen Teilchenoberflächen die metallorganische Verbindung haftet, durch Plasmaerwärmung, um einen kalzinierten Körper zu erhalten, in dem Metalloxide von M reduziert sind, die an in der metallorganischen Verbindung enthaltenem O gebunden sind;
Verdichten des kalzinierten Körpers, um einen verdichteten Körper zu erhalten;
Sintern des verdichteten Körpers,
wobei der Permanentmagnet auf Nd-Fe-B basiert, und
der Permanentmagnet Nd in einem Bereich von 25 bis 37 Gew.%, Fe in einem Bereich von 60 bis 75 Gew.% und B in einem Bereich von 1 bis 2 Gew.% enthält.

2. Herstellungsverfahren für einen Permanentmagneten, umfassend folgende Schritte:
Mahlen von Magnetmaterial zu Magnetpulver;
Zugeben einer metallorganischen Verbindung, ausgedrückt durch eine Strukturformel
M-(OR)ₙ
wobei M V, Mo, Zr, Ta, Ti, W oder Nb darstellt, R eine Substituentengruppe darstellt, die aus einem geradkettigen oder verzweigtkettigen Kohlenwasserstoff besteht, und n die Wertigkeit des Metalls oder Metalloids darstellt;
zu dem Magnetpulver, das bei dem Mahlschritt von Magnetmaterial erhalten wurde, und Anhaftenlassen der metallorganischen Verbindung an Teilchenoberflächen des Magnetpulvers;
Verdichten des Magnetpulvers, an dessen Teilchenoberflächen die metallorganische Verbindung haftet, um einen verdichteten Körper zu erhalten,
**dadurch gekennzeichnet, dass** das Herstellungsverfahren ferner folgende Schritte aufweist:
Kalzinieren des verdichteten Körpers durch Plasmaerwärmung, um einen kalzinierten Körper zu erhalten, in dem Metalloxide von M reduziert sind, die an in der metallorganischen Verbindung enthaltenem O gebunden sind;
Sintern des kalzinierten Körpers,
wobei der Permanentmagnet auf Nd-Fe-B basiert, und
der Permanentmagnet Nd in einem Bereich von 25 bis 37 Gew.%, Fe in einem Bereich von 60 bis 75 Gew.% und B in einem Bereich von 1 bis 2 Gew.% enthält.

3. Herstellungsverfahren für einen Permanentmagneten nach Anspruch 1 oder 2, wobei der kalzinierte Körper bei dem Kalzinierungsschritt durch Erwärmung mittels Wasserstoffplasma bei hoher Temperatur erhalten wird.

4. Herstellungsverfahren für einen Permanentmagneten nach einem der Ansprüche 1 bis 3, wobei das Magnetmaterial bei dem Mahlschritt von Magnetmaterial zu Magnetpulver gemahlen wird, um Magnetpulver mit der Teilchengröße einer Einzeldomäne zu erhalten.

5. Herstellungsverfahren für einen Permanentmagneten nach einem der Ansprüche 1 bis 4, wobei R in der Strukturformel eine Alkylgruppe ist.

6. Herstellungsverfahren für einen Permanentmagneten nach Anspruch 5, wobei R in der Strukturformel eine Alkylgruppe ist, deren Kohlenstoffzahl irgendeine der Ganzzahlen 2 bis 6 ist.

## Revendications

1. Procédé de fabrication d'un aimant permanent, comprenant les étapes suivantes :
broyage d'un matériau d'aimant pour constituer une poudre d'aimant ;
ajout d'un composé organométallique répondant à la formule structurelle
M-(OR)ₙ
M représentant V, Mo, Zr, Ta, Ti, W ou Nb, R représentant un groupe substituant constitué par une chaîne hydrocarbure droite ou ramifiée, et n représentant la valence du métal ou métalloïde, à la poudre d'aimant obtenue à l'étape de broyage du matériau d'aimant ; et
réalisation d'une adhésion du composé organométallique aux surfaces des particules de poudre d'aimant ;
**caractérisé en ce que** le procédé de fabrication comprend en outre les étapes suivantes :
calcination de la poudre d'aimant dont les surfaces de particule présentent une adhésion au composé organométallique par chauffage au plasma de manière à obtenir un corps calciné dans lequel des oxydes métalliques de M qui ont été liés avec l'O contenu dans le composé organométallique composé sont réduits ;
compactage du corps calciné de manière à obtenir un corps compact ; et
frittage du corps compact,
dans lequel l'aimant permanent est basé sur Nd-Fe-B, et
l'aimant permanent comprend du Nd dans une plage de 25 % à 37 % en masse, du Fe dans une plage de 60 % à 75 % en masse, et du B dans une plage de 1 % à 2 % en masse.

2. Procédé de fabrication d'un aimant permanent, comprenant les étapes suivantes :
broyage d'un matériau d'aimant pour constituer une poudre d'aimant ;
ajout d'un composé organométallique répondant à la formule structurelle
M-(OR)ₙ
M représentant V, Mo, Zr, Ta, Ti, W ou Nb, R représentant un groupe substituant constitué par une chaîne hydrocarbure droite ou ramifiée, et n représentant la valence du métal ou métalloïde, à la poudre d'aimant obtenue à l'étape de broyage du matériau d'aimant ; et
réalisation d'une adhésion du composé organométallique aux surfaces des particules de poudre d'aimant ;
compactage de la poudre d'aimant dont les surfaces de particule présentent une adhésion au composé organométallique de manière à obtenir un corps compact ;
**caractérisé en ce que** le procédé de fabrication comprend en outre les étapes suivantes :
calcination du corps compact par chauffage au plasma de manière à obtenir un corps calciné dans lequel des oxydes métalliques de M qui ont été liés avec l'O contenu dans le composé organométallique composé sont réduits ; et
frittage du corps calciné,
dans lequel l'aimant permanent est basé sur Nd-Fe-B, et
l'aimant permanent comprend du Nd dans une plage de 25 % à 37 % en masse, du Fe dans une plage de 60 % à 75 % en masse, et du B dans une plage de 1 % à 2 % en masse.

3. Procédé de fabrication d'un aimant permanent selon la revendication 1 ou 2, dans lequel le corps calciné est obtenu à l'étape de calcination par un chauffage au plasma d'hydrogène à haute température.

4. Procédé de fabrication d'un aimant permanent selon l'une quelconque des revendications 1 à 3, dans lequel, à l'étape de broyage du matériau d'aimant, le matériau d'aimant est broyé en poudre d'aimant de manière à obtenir une poudre d'aimant présentant une taille de particule de domaine unique.

5. Procédé de fabrication d'un aimant permanent selon l'une quelconque des revendications 1 à 4, dans lequel R dans la formule structurelle est un groupe alkyle.

6. Procédé de fabrication d'un aimant permanent selon la revendication 5, dans lequel R dans la formule structurelle est un groupe alkyle dont le nombre d'atomes de carbone est un entier quelconque compris entre 2 et 6.
